

## UNITED STATES PATENT OFFICE.

FREDERICK C. STANLEY, OF BRIDGEPORT, CONNECTICUT, ASSIGNOR TO RAYBESTOS COMPANY, OF BRIDGEPORT, CONNECTICUT, A CORPORATION OF CONNECTICUT.

## PROCESS OF MAKING FRICTION FACINGS AND PRODUCT.

No Drawing. Application filed September 24, 1919, Serial No. 325,913. Renewed October 28, 1921. Serial No. 511,103.

To all whom it may concern:

Be it known that I, FREDERICK C. STANLEY, a citizen of the United States, residing in the city of Bridgeport, county of Fairfield, and State of Connecticut, have invented certain new and useful Improvements in Processes of Making Friction Facings and Products, of which the following is a specification.

10 This invention relates to improvements in process of making friction facings and refers more particularly to a clutch facing or brake lining adapted for use in motor vehicles.

15 The invention is directed to a novel process of making a friction facing from felted unwoven asbestos fibre saturated with a binder.

20 The object of the invention is to provide a process by which the friction facing has a maximum tensile strength and hardness so that it can withstand the shocks to which these facings are subjected in a motor car and also will have sufficient resistance to 25 abrasion; while at the same time it has the proper coefficient of friction. It is also necessary that the binder in these facings must be unaffected by oil or water in use, which object is accomplished by the present 30 invention without in any way detracting from the other characteristics.

The process may be carried out as follows: asbestos fibre preferably the short or low grade fibre is first ground in a suitable 35 grinding machine or cutter. The ground material is then put into a beater mixed with the water or other solution and beaten into a pulp. The pulp is then delivered to a paper making machine as for example a 40 wet board machine and formed into sheets or boards of suitable width and thickness. This forms an unwoven felted sheet.

45 As a feature of the invention, there is added to the pulp in the beater, very finely comminuted graphite. This graphite is added for the purpose of making a smooth sheet and to increase the ability of the finished product to resist attrition or abrasion either from action of grit on the fac- 50 ing in operation or from scoring from the metal bearing surface. This graphite is added in proportion by weight of from four tenths of one percent to five percent of the dry asbestos fibre. The amount of graphite 55 used depends upon the co-efficient of fric-

tion desired. In other words, if the co-efficient of friction must not be materially affected the minimum amount of graphite is used. If the co-efficient of friction however is not so important, the larger amount 60 may be used and even more than five percent may be used. There is also mixed with the pulp in the beater an oxidizing agent, as for example red oxide of lead. In using red lead as an oxidizing agent, the amount 65 employed is approximately 1.6 percent by the weight of the asbestos fibre although this can be varied according to the characteristics of the product desired. This oxidizing agent facilitates or hastens the cure 70 of the binder and adds to the strength of the product and also converts the binder into a form insoluble by oil or water. It also tends to produce a uniform curing 75 throughout the mass during the curing operation hereinafter described. It is to be noted that this reagent is put into the pulp before the formation of the sheet and not during the saturating and curing steps of 80 the process.

85 After the sheets or boards have been formed as described, they are subjected to hydraulic pressure in suitable presses and are then hung up to dry in a drying room of sufficient temperature to remove the wa- 90 ter. The sheet is then calendered to the desired thickness and the friction facings are then cut out of the sheet. The sheets are subjected to sufficient pressure in the calender to obtain as much tensile strength 95 in the dry sheet as is feasible. The friction facings whether clutch rings or brake linings are now ready for saturation. The saturating tank is filled with a binder. This binder may consist of 94 percent of lin- 100 seed oil, 6 percent of gilsonite in the solution in the oil thinned with gasoline to about 33 Baumé gravity. The friction facings are then immersed while suspended on suitable rods in this binder solution for a 105 period of half an hour. The friction facings are then removed and put in a closed steam oven and maintained at a temperature of about 200° F. to drive off the gasoline which gasoline may be recovered and saved. This steam treatment is preferably continued from two to three hours. The friction facings are then removed to a closed baking oven where they are subjected to a tem- 110 perature of about 250° F., for a period of

twelve hours. The facings are then taken out of the oven and immersed in another saturating tank containing a solution of 66 percent of linseed oil and 33 percent of gasoline, the gravity of the solution being about 33 Baumé. This second immersion takes place for from two to three minutes. In both of the saturating steps double boiled linseed oil is preferable.

10 The friction facings are then put into a second closed baking oven and maintained at a temperature of 300° F. for twenty-four hours. The heat in both of the baking ovens is preferably dry heat. The friction facings are then removed from the second oven and sand papered to micrometer size and to get a smooth finish to the facing. The facings are now ready for use.

15

I have given above an illustration in 20 which the process is actually carried out in commercial operation. It is to be understood that the temperature and length of treatment are subject to reasonable variations depending on the flexibility and 25 strength required in the finished product. Also oils other than linseed oil may perhaps in certain cases be used and other asphalts substituted for gilsonite.

During the baking operation, the linseed 30 oil, due to the presence of the air in the oven and also to the oxidizing agent of the sheet is oxidized to produce a tough hard binder. The solubility of the linseed oil in the gasoline before the baking treatments is practically 35 100% while after the baking treatments it is very materially reduced; and in fact the baking operation may be so carried out as to make the oil practically insoluble in the gasoline. It is to be noted that by means 40 of the double saturation and double baking, a more efficient curing of the binder is obtained and the sheet can be impregnated with larger quantities of binder. This adds greatly to the tensile strength and hardness 45 of the finished product. In order that the tensile strength of the friction facings made in this manner may be more clearly understood, I submit the following table giving actual tests made on such friction facings:

50

55

60

| Thickness of sheet before calendering in inches | Thickness of sheet after calendering in inches | Average tensile strength of finished facing in pounds per square inch | Average hardness of finished facing by Brinell test |
|-------------------------------------------------|------------------------------------------------|-----------------------------------------------------------------------|-----------------------------------------------------|
| .150                                            | .123                                           | 4614                                                                  | 23.4                                                |
| .145                                            | .123                                           | 4282                                                                  | 17.2                                                |
| .140                                            | .123                                           | 4028                                                                  | 16.6                                                |
| .135                                            | .123                                           | 3966                                                                  | 15.3                                                |

The strength and hardness of the product made by this process is far in excess, in fact from 1000 to 2000 lbs., upwards in tensile

strength, over that heretofore obtained from any unwoven saturated friction facing and 65 is even stronger than a woven sheet. The hardness also is proportionately increased over the friction facings heretofore made. It is to be noted that in the baking operation, the reaction develops autogenous heat 70 or in other words exo-thermic and care must be taken to prevent the material from becoming so highly heated as to catch fire. This exo-thermic reaction results in the fact that the oxidation is of such a character as 75 to generate heat in addition to that externally applied. This exo-thermic reaction of oxidation is well known in other arts as for example in the manufacture of air blown asphalt from petroleum residuum. 80

I claim as my invention:

1. A process of making a friction facing, of mixing asbestos pulp with an oxidizing agent and with comminuted graphite, forming sheets therefrom, cutting friction facings from the sheets, saturating the facings with a binder oil and baking the friction facings. 85

2. A process of making a friction facing consisting in mixing asbestos pulp with 90 comminuted graphite, forming unwoven sheets therefrom, cutting friction facings from such sheets and subjecting the friction facing to a saturation in a binder oil and then baking. 95

3. A friction facing, the wearing surface of which consists essentially of unwoven asbestos fibre, a baked binder and graphite.

4. The process of making friction facings, consisting in incorporating with fibrous material a comminuted graphite, saturating the same in a binder and then baking the facing. 100

5. The process of making friction facings, consisting in incorporating with fibrous material a comminuted graphite, in saturating the facings with an oil, and in then baking said facings containing the comminuted graphite and the oil. 105

6. The process of making friction facings, 110 consisting in mixing fibrous pulp with graphite and forming unwoven sheets therefrom, saturating the facing with a binder oil, and then baking the facing.

7. The process of making friction facings, 115 consisting in mixing asbestos with a comminuted graphite, saturating the asbestos with a binder oil and subjecting the saturated material to heat treatment.

8. The process of making friction facings, 120 consisting in mixing fibrous pulp with a comminuted graphite, forming sheets therefrom, saturating the sheet with a binder oil, and subjecting the saturated sheets to heat treatment.

FREDERICK C. STANLEY.